

# UNITED STATES PATENT OFFICE.

SEBASTIANO RANNO FU BIAGIO, OF NEW YORK, N. Y.

## BUILDING-BLOCK.

1,081,695.

Specification of Letters Patent.

Patented Dec. 16, 1913.

No Drawing.

Application filed July 30, 1912. Serial No. 712,358.

*To all whom it may concern:*

Be it known that I, SEBASTIANO RANNO FU BIAGIO, a citizen of the United States, residing at New York, in the county of New York and State of New York, have invented certain new and useful Improvements in Building-Blocks, of which the following is a specification.

My invention relates to blocks adapted for use in buildings, paving and the like, and has for its object the provision of an improved block and the composition thereof by which the block is of a glazed character and exceedingly hard and tough, and likewise practically impervious to fire.

In making my improved block I use pulverized granite 20 parts, pulverized glass 10 parts, and 35 parts each of fire clay and red clay thoroughly mixed together and fused by means of heat, the temperature to which the ingredients are subjected being upward of 1500 degrees Fahrenheit. Prior to baking the blocks I mix with the clay, pulverized granite and glass, (1%) one per cent. of the entire mixture of bicarbonate of soda. It will be understood that the bicarbonate of soda forms a flux to assist in the melting of the pulverized granite and pulverized glass, as well as lowering the fusing point of the other ingredients, and that the pulverized granite and the pulverized glass render the blocks when finished very durable and furthermore, gives the blocks a glazed and ornamental appearance, while the red clay after being baked as heretofore stated turns the mass to a black color, and the fire

clay makes the blocks impervious to heat of less than 1500 degrees Fahrenheit. It will also be understood that by the use of bicarbonate of soda a block is made that is exceptionally hard and tough; and because of the thorough fusing of all the parts during the baking process the block is a good resistant of heat.

If it is desired to produce a block which is very refractory, the red clay may be dispensed with and a larger amount of fire clay used, and on the other hand if the heat resisting quality of the block desired is immaterial, the fire clay may be dispensed with and a larger amount of red clay used.

It will, of course, be understood that the proportions of the various ingredients may be varied greatly from those above stated, without departing from the scope or spirit of the invention as claimed.

Having thus described my invention what I claim is:—

A process for manufacturing building blocks by mixing 20 parts of pulverized granite, 10 parts of pulverized glass, 35 parts of red clay, 35 parts of fire clay and bicarbonate of soda in an amount equaling 1 per cent. of the entire mixture, and fusing the entire mixture by means of a high temperature.

his  
SEBASTIANO X RANNO FU BIAGIO.  
mark

Per B. RANNO.

Witnesses:

LUDOVICO FERRIRI,  
LUCIDO BAMONTI.